

F. SCHWARTZ.  
TOE OR HEEL STIFFENER.  
APPLICATION FILED APR. 17, 1915.

1,215,876.

Patented Feb. 13, 1917.



INVENTOR.

Frank Schwartz  
By his Attorney  
Nelson M. Howard

# UNITED STATES PATENT OFFICE.

FRANK SCHWARTZ, OF WINTHROP, MASSACHUSETTS, ASSIGNOR TO UNITED SHOE MACHINERY COMPANY, OF PATERSON, NEW JERSEY, A CORPORATION OF NEW JERSEY.

## TOE OR HEEL STIFFENER.

1,215,876.

Specification of Letters Patent. Patented Feb. 13, 1917.

Original application filed January 26, 1915, Serial No. 4,466. Divided and this application filed April 17, 1915. Serial No. 22,116.

To all whom it may concern:

Be it known that I, FRANK SCHWARTZ, a citizen of the United States, residing at Winthrop, in the county of Essex and State 5 of Massachusetts, have invented certain Improvements in Toe or Heel Stiffeners, of which the following description, in connection with the accompanying drawings, is a specification, like reference characters on 10 the drawings indicating like parts in the several figures.

This invention relates to stiffeners for boots and shoes; and the present application is a division of co-pending application Serial No. 4466.

It has been common hitherto in the manufacture of boots and shoes either to apply a stiffening substance such as box-toe gum in a liquid or plastic state to the box-toe 20 blank when the upper is assembled or to assemble with the upper a normally stiff box-toe blank which is capable of being softened by heat. In the first case the upper is immediately pulled over and lasted 25 while in the second case the stiff blank is steamed before each operation so as to soften it temporarily. In either case, after the lapse of a certain amount of time the box-toe becomes hard. The use of box-toe gum 30 is objectionable for many reasons and has been supplanted to a considerable extent by the normally stiff blank which is adapted to be softened by heat. There are, however, serious objections to the use of this normally stiff blank. It is desirable to fasten 35 this blank to the upper by stitches, but because of the stiffness of the blank the needles of the sewing machine, by which the stitching is done, are frequently bent or broken. Again this prepared blank, as has been 40 stated, requires two steamings one before the pulling-over operation and one before the lasting operation, since it becomes stiff very rapidly when removed from the steaming 45 apparatus. Moreover a blank of this kind is bulky and this, together with its quality of stiffening quickly, has an injurious effect on the lasting operation so that it is difficult to produce a smooth toe on the finished shoe. 50 Indeed it is customary when this normally stiff blank is used, to rub out the bunches at the toe by pressing the toe against a highly heated iron so as to soften the stiffening material and smooth out the bunches.

One feature of the present invention comprises a suitably shaped blank of sheet material carrying particles of a stiffening material which is normally hard but may be softened by the application of heat. 55

This and other features of the invention 60 will be described in connection with an illustrative article and pointed out in the appended claims.

Referring now to the accompanying drawing, 65

Figure 1 is a perspective of a stiffener in which the present invention is embodied, one of the plies of fabric having been bent back to show the powdered or granulated 70 stiffening material.

Fig. 2 is a section of the fore part of a shoe in which the stiffener has been embodied.

In the illustrative embodiment of the invention the box-toe blank indicated as a 75 whole at 1 is made of two pieces or plies of fabric 2, 3, and between the plies is a layer or coating 5 of a powdered or granulated material, such for example as shellac, the melting point of which is comparatively low 80 so that the stiffening material may be melted or softened by a heat which will have no injurious effect upon the leather.

In order to hold the powdered or granulated shellac securely, an adhesive of some 85 sort may be used; and in the illustrative embodiment of the invention the fabric of the box-toe blank is the well-known "backing cloth" which is commonly used to strengthen the uppers of boots and shoes, this backing 90 cloth consisting of a piece of fabric having on one face a coating of adhesive containing gutta-percha. To prepare a box-toe blank a suitable amount of powdered or granulated shellac is dusted or sprinkled on the 95 coated side of a sheet of the backing cloth and then a second sheet is pressed upon the first sheet with the coated sides together after which the blank is dried out.

In order to prevent the melted or softened shellac from penetrating the lining of the shoe during the subsequent heating operation a sheet of paper 12 or other impervious substance may be applied to the box-toe blank on one or both sides. 100

In the manufacture of a shoe the blank may be incorporated in the upper between the lining 8 and the toe tip 10 in any suit- 105

able manner, as, for example, by the row of stitches, one of which is shown at 7, which unites the tip 10 to the vamp. The upper is then assembled on the last and the pulling-over and lasting operations carried out while the blank is in its normal condition and the stiffening material still in its powdered or granulated or broken state. The blank at this time is still flexible. In order 10 to complete the formation of the box-toe and set the blank the forward portion of the lasted shoe is placed in a suitable heating apparatus such, for example, as that shown in British Patent No. 13155 of 1910 and subjected to a heat sufficient to soften or melt 15 the shellac whereby the particles of shellac are caused to run together and to permeate the fabric of the box-toe blank so that when the shellac hardens a finished box-toe is produced.

When the upper is lasted the toe of the upper, together with the box-toe blank, is drawn tightly about the toe of the last, the leather being put under considerable tension. Consequently if there are any bunches 25 due to the presence of too much powdered or granulated shellac at any points the strain of the leather smooths out such bunches when the shellac softens or melts, so that the resulting box-toe is smooth and conforms to 30 the form of the toe of the last.

I have found that by subjecting the toe of the shoe for approximately an hour to a temperature of between 210° and 250° F. a 35 box-toe for the making of which two pieces of backing cloth and a layer of powdered shellac are used, is hard when taken out of the heating apparatus so that if desired the last may be pulled at once. I have also 40 found that this hardness is permanent to the extent that further heat for the same time at the same temperature will not appreciably affect it. In any event, however, softened shellac when removed from a temperature 45 of from 210° to 250° to the ordinary temperature of a shoe factory will harden in a few minutes. The important effect of this heating operation is to soften and amalgamate the shellac and cause it to permeate 50 the fabric so that whereas before the heating it is in the form of separated masses or particles after the heating it forms a more or less continuous film which serves to give permanent form to the toe of the shoe.

Throughout the specification the stiffening material referred to has been powdered or granulated shellac. This has been done, however, to promote brevity. Any suitable substance may be used which will permit the 60 blank to be flexible normally so as not to interfere with the lasting operation and at the same time may be subsequently melted or softened so as to complete the formation of the box. And whether the stiffening material is strictly in powdered or granulated

form is obviously immaterial so long as the normal flexibility of the blanks and its capability of being subsequently softened and set are present. For example the shellac may be applied to the fabric in solution and 70 allowed to stiffen after which the prepared fabric may be run through a mangle to break up the shellac and render the product flexible. The manner in which the blank is incorporated in the upper is also immaterial. 75 For example, instead of being stitched to the upper it may be cemented or merely laid in. And although the article has been described as a box-toe blank and the method as one which results in the production of a box-toe it should be understood that the invention is applicable to any sort of stiffener such for example as a counter.

Having thus described my invention, what I claim and desire to secure by Letters Patent of the United States is:

1. A stiffener for parts of boots and shoes consisting of a suitably shaped blank comprising a piece of fabric coated with separated particles of a stiffening material which is normally hard but may be softened by the application of heat, of a degree insufficient to injure the shoe part.

2. A stiffener for parts of boots and shoes consisting of a suitably shaped blank comprising a piece of fabric, a coating of adhesive substance and a layer of powdered or granulated stiffening material which is normally hard but may be softened by the application of heat, of a degree insufficient to injure the shoe part.

3. A stiffener for parts of boots and shoes consisting of a suitably shaped blank comprising two pieces of fabric and a layer of powdered or granulated stiffening material held between them, said material being capable of being fused by a degree of heat insufficient to injure the shoe part.

4. A stiffener for parts of boots and shoes consisting of a suitably shaped blank comprising a piece of fabric and a stiffening material in solid broken state carried thereby, said material being capable of being fused by a degree of heat insufficient to injure the shoe part.

5. A stiffener for parts of boots or shoes consisting of a suitably shaped normally flexible blank comprising a piece of fabric coated with dry particles of a stiffening material which is normally hard but may be softened by the application of heat, of a degree insufficient to injure the shoe part.

6. A stiffener for parts of boots and shoes consisting of a suitably shaped blank comprising two pieces of fabric, a coating of adhesive containing gutta-percha, and a layer of powdered or granulated shellac held in place by said adhesive.

7. A stiffener for parts of boots and shoes consisting of a suitably shaped blank of

sheet material, an adhesive substance thereon, and separated particles of a stiffening material held in place by said adhesive substance, said stiffening material being capable 5 of being softened by a degree of heat insufficient to injure the shoe part.

8. A stiffener for parts of boots and shoes consisting of a suitably shaped blank comprising a piece of sheet material, and a stiffening material in solid, broken state carried thereby, said stiffening material being capable of being softened by a degree of heat 10 insufficient to injure the shoe part.

9. A stiffener for parts of boots and shoes consisting of a suitably shaped blank comprising a piece of fabric, a stiffening material in solid, broken state carried thereby, said material being capable of being softened by a degree of heat insufficient to injure the shoe part, and a piece of sheet ma- 15 terial impervious to the softened stiffening material.

In testimony whereof I have signed my name to this specification.

FRANK SCHWARTZ.